

## UNITED STATES PATENT OFFICE

GEORGE A. RICHTER AND MILTON O. SCHUR, OF BERLIN, NEW HAMPSHIRE, ASSIGNORS  
TO BROWN COMPANY, OF BERLIN, NEW HAMPSHIRE, A CORPORATION OF MAINE

## FIBER-LIBERATING PROCESS

No Drawing.

Application filed June 27, 1927. Serial No. 201,957.

This invention involves the liberation of fiber from raw cellulosic materials, particularly woods of high resin content such as heretofore considered inferior raw material 5 for the production of pulp.

In producing pulp from woods of resinous character, alkaline processes of digestion have generally been found more satisfactory than the sulphite process, as the alkali reacts 10 with and dissolves not only the ligneous components of the wood but also a certain amount of the resinous components. There are certain woods so rich in resin, however, that even alkaline digestion does not produce a 15 pulp of suitable quality, the resin content being sufficiently reacted upon and removed by the alkali. This doubtless may be ascribed to the fact that the resin content of wood comprises resins both of a saponifiable character and inert resins, perhaps of the nature 20 of polymerized hydrocarbons which survive alkaline digestion and are present in considerable quantity in the resulting pulp. Such residual resins when present in a pulp 25 tend to clog and gum washing cylinders and thickeners and raise havoc with the wires and felts of papermaking machinery, so that woods rich in resin, such as jack pine, although found in abundance, have been employed only to a limited extent for the 30 production of pulp.

We have found that if soap is present in the usual alkaline digesting liquors, the difficulties heretofore encountered when woods of 35 even a highly resinous character are employed as a raw material are largely eliminated, and a softer pulp having good papermaking qualities produced. While we are unable to account precisely for these results, 40 it is quite likely that the soap component of the digesting liquor disperses or colloidally dissolves unsaponifiable or difficultly saponifiable resins which the alkali cannot react with and dissolve.

A procedure such as described permits the 45 use of soap-forming substance rather than previously prepared soap, as soap may be readily produced in situ in the digester while digestion is taking place. Furthermore, the 50 action of the soap upon the resins facilitates

the resolution of the chips into fiber. The soaps which we employ may be straight-chain, fatty acid soaps such as sodium oleate, sodium palmitate or sodium stearate, or ring-structure soaps such as rosin soap or the 55 soaps of sulphonated oils. As soap-forming substance, we may employ oils or fats such as palm oil, coconut oil, peanut oil, or other fatty acid glycerides or fatty acids which would saponify readily under the conditions 60 prevailing during digestion to produce soap.

In practising the process of the present invention, we may proceed along the same general lines followed when practising usual alkaline digestion, but the wood employed as raw material may be of a resinous or highly 65 resinous character, such as jack pine. The wood is chipped and then charged into a digester of the usual type employed for alkaline digestion, whereupon the alkaline liquor desired is run into the digester. The liquor may be the so-called sulphate liquor consisting essentially of a solution of caustic 70 soda and sodium sulphide, or the so-called soda liquor consisting essentially of a solution of caustic soda only. To the liquor is then added sufficient soap or soap solution to produce a soap concentration of 0.3% to 0.4%, based on liquor. The soap concentration may 75 be varied, however, depending upon the resin content of the particular wood employed as a raw material, and the extent to which it is desired to deresinify the pulp. In lieu of adding a prepared soap, we may add soap-forming substance, such as palm oil, in 80 amount sufficient to produce the desired soap concentration, and when this is done, the caustic soda content of the liquor is preferably sufficiently in excess of the usual content to allow for the saponification of such soap-forming substance. The charge is then digested under pressure and at elevated temperature until a fiber liberation has been effected, as is customary in alkaline digestion.

During digestion, the alkali exerts its usual function of dissolving the encrusting material from the wood and at the same time the soap reacts upon and disperses resins which are not reacted on by the alkali and which otherwise would be present in the re- 100

sulting pulp. If soap-forming substance has been added, saponification of such substance takes place quite readily as digestion proceeds, producing soap in situ and effecting the desired deresinification of the pulp. The soap greatly assists the alkali in softening the fiber and in promoting a fiber liberation from the chips. It also effects a detergent effect upon the smaller non-resinous particles 5 usually present in pulp, particularly alkaline-digested pulp, and enhances the bleachability of such pulp.

10 After digestion, the pulp may be separated from the spent liquor, as by passing such pulp through a washer as usual. Inasmuch as the pulp has been deresinified during digestion, no difficulty is experienced due to gumming of the washing cylinders; nor does such pulp do mischief to thickeners or papermaking 15 machinery with which it subsequently contacts.

15 The separated spent liquor may be subjected to recovery processing such as usually practised in connection with alkaline digestion. The spent liquor is of higher organic or combustible content than usual, owing to the removal of resins from the wood and the fatty acid grouping of the soap, and hence when concentrated and incinerated in a combined boiler-smelter furnace for the recovery of its valuable sodium constituent gives a higher fuel value than ordinarily. The recovery of sodium constituent previously present in the digesting liquor in the 20 form of soap and fiber-liberating chemical may thus be effected in one operation.

25 When a highly resinous wood such as jack pine is employed as a raw material, peptizing agents such as sodium phosphate, borax, talc, or colloidal clay may be employed to good advantage in the digesting liquor, together with the soap, to assist in deresinifying the pulp.

30 By the process of the present invention, woods of high resin content may be converted into pulp satisfactory for papermaking. While deresinification might be accomplished by suitable treatment of pulp after its removal from the digester, as described in our application, Serial No. 202,454, filed June 29, 1927, nevertheless deresinification in the digester is preferable in the case of highly resinous woods, as the resins are removed before they contact with apparatus to which 35 they might do injury. The apparatus, power, and time incident to the practice of our process is practically the same as that necessary in usual alkaline digestion, and the valuable sodium constituent of the soap may be re-covered along with the sodium constituent of the fiber-liberating chemicals. Furthermore, deresinification is accomplished under very favorable conditions, as under the influence of heat and pressure such as prevails during digestion, the resin content is

believed to exist in a softened or plastic condition, permitting very effective action by the soap.

Having thus described our invention, it is evident to those skilled in the art that various changes might be resorted to without departing from its spirit or scope as defined in the appended claims.

What we claim is:

1. A fiber-liberating process which comprises digesting chipped wood under pressure and at elevated temperature in an alkaline liquor of a saponaceous character.

2. A fiber-liberating process which comprises digesting chipped wood under pressure and at elevated temperature in an alkaline liquor containing soap and a peptizing agent.

3. A fiber-liberating process which comprises digesting chipped jack pine under pressure and at elevated temperature in an alkaline liquor containing soap.

4. A process which comprises digesting a resinous wood under pressure and at elevated temperature in an alkaline liquid containing sodium base compounds and a sodium base soap, separating the spent liquor from the resulting pulp, and recovering the sodium constituent from the spent liquor.

5. A fiber-liberating process which comprises digesting chipped wood in an alkaline liquor containing about 0.3% to 0.4% soap, based on liquor.

6. A fiber-liberating process which comprises digesting wood under pressure and at elevated temperature in an alkaline liquor containing a soap-forming substance and sufficient caustic soda to saponify such substance and to effect a liberation of fiber from such wood.

7. A fiber-liberating process which comprises digesting chipped wood under pressure and at elevated temperature in an alkaline liquor containing a fatty acid glyceride and sufficient caustic soda to saponify the glyceride and effect a liberation of fiber from such wood.

In testimony whereof we have affixed our signatures.

GEORGE A. RICHTER. 115  
MILTON O. SCHUR.

70

80

85

90

95

100

105

110

115

120

125

130